

## UNITED STATES PATENT OFFICE

JEAN GEORGES KERN AND CHARLES J. SALA, OF WILMINGTON, DELAWARE, ASSIGNORS  
TO E. I. DU PONT DE NEMOURS & COMPANY, OF WILMINGTON, DELAWARE, A COR-  
PORATION OF DELAWARE

## VAT ASSISTANT FOR USE IN DYEING

No Drawing.

Application filed August 4, 1927. Serial No. 210,715.

This invention relates to the art of dyeing and more particularly to the preparation and application to cellulose or artificial silk fabrics of a dyeing bath containing a material adapted to facilitate the dyeing operation. The invention also relates to the dyeing liquor and to the fabric dyed therewith as articles of manufacture.

As is well understood in the art, by the term "vat dye" is meant a coloring matter insoluble in water but which can be converted on reduction into a so-called leuco-compound which is soluble to a certain extent in solutions of alkali. Such vat dyes are characterized by their excellent fastness but the difficulty of dyeing them satisfactorily with fair yield has been a drawback to their use in this connection. One of the objects of the present invention is to overcome this difficulty 20 in the manner described in detail below.

In dyeing with vat colors as carried out at present several processes are followed:

1. On piece goods.
  - a. Jigger dyeing method.
  - b. Padding method in reduced bath.
  - c. Padding method in unreduced bath with subsequent development of the dye in jigger. This process is the most usually adopted.
2. Dyeing of raw-stock, unspun cotton, in machine.
3. Dyeing of yarn on beams or packages in machines.

In general this invention relates in all or some of its improvements to the operation of dyeing cotton or artificial silk fibres in any of these ways.

Most of these processes require the use of a reduced bath. To undergo this operation the vat dyestuff is generally passed through a fine screen (200 mesh/inch) diluted somewhat with water and added to the dyebath containing a corresponding amount of alkali and a reducing agent such as sodium hydro-sulfite, which is the most commercially used. The temperature is raised for this purpose to a suitable point according to the particular vat dyestuff used and when complete reduction is reached the dyeing operation is started.

It is essential that all during the dyeing operation the dye be kept in its most highly dispersed state.

Therefore, it is first of all important that the dyestuff paste be of special fineness but even with the finest pastes at present in commerce a great deal of color is lost because of its failure to dye the fibre. This wasted dyestuff is, in many cases not taken up by the fibre, and washes off during the soaping operation which follows the dyeing. Also, in most cases the great affinity of the reduced dyestuff itself for the fibre is a handicap to producing even dyeings.

Now we have found, however, that certain organic compounds, when mixed either with the dyestuff paste or when dissolved in the dyebath, produce various improved results. These organic compounds are not in themselves new but it is believed that the use of them for this purpose is entirely new. The compounds we employ are substituted aliphatic amines containing hydroxyl groups in the aliphatic radicals. They are very strongly basic and possess a high degree of solubilizing power.

The general formula for substances of this class is:



R<sub>1</sub>, R<sub>2</sub> representing either an alkyl group C<sub>n</sub>H<sub>(2n+1)</sub> hydrogen, or a hydroxy alkyl group C<sub>n</sub>H<sub>2n</sub>OH. It makes no difference whether R<sub>1</sub> is hydrogen while R<sub>2</sub> is an alkyl group or R<sub>2</sub> is hydrogen and R<sub>1</sub> an alkyl group. Also any one of these substituents already described may be replaced by a compound containing the group C<sub>n</sub>H<sub>(2n-1)</sub>(OH)<sub>2</sub>. 85 90

In carrying our invention into effect we can proceed in two ways.

1. We may mix the ingredient adopted to facilitate the dyeing operation into the vat color paste, dilute somewhat with water, and pass this suspension through a screen as described above. This suspension which is very highly dispersed is then added to the dyebath containing the alkali and the reducing agent. The temperature is then brought to about the 100

appropriate dyeing temperature at the start. A complete reduction followed by a complete solubilization of the leuco is the result. The chemical process is not essentially different from one method to the other, except when 5 pad-method is used. In this case the unreduced dyestuff is mixed with the assistant as outlined above then diluted to a certain concentration with water, gum and oil, the material padded therewith and dried and later 10 developed on a jigger in a solution as described above and composed of alkali and a reducing agent. Additional dyestuff may or may not be added in this case.

15 After the dyeing operation which takes about 45 minutes the material is rinsed and treated with an oxidizing agent such as bichromate of soda, or preferably perborate of soda, rinsed and thoroughly soaped, then 20 again rinsed, allowed to dry and finished.

25 The presence of the new assistant very effectively aids the transfer of the dye to the cotton and a number of advantages are obtained.

30 2. We may also use the vat color pastes prepared in the manner described in our co-pending application, Serial No. 167,066, which pastes already contain the new assistant, the dyeing process being hence not different from the ordinary vat color dyeing processes, with the exception that the results are obtained as according to the present invention.

In order fully to disclose our process the 35 following examples of typical dyebaths and methods are furnished.

It is to be understood, however, that these examples are only illustrative and that the conditions, proportions and reagents specified therein may be varied within wide limits, 40 that is:

#### EXAMPLE I

An 8½% shade of Ponsol blue GD (Schultz #842) on 150 lbs. of mercerized cotton piece 45 goods is obtained as follows:

12.75 lbs. of Ponsol blue GD (Schultz #842) are mixed with

8.16 lbs. of the new dye assistant

50 1 gal. of cold water added and the suspension passed through a fine screen. A perfect speckless paste is so obtained which is added to the jigger dyebath, composed of the following:

55 10 lbs. caustic soda

15 lbs. hydrosulfite conc. 10 lbs. added immediately, 5 lbs. after 1 passage.

100 gals. water.

60 The temperature raised to 110° F., and after complete reduction the dyeing started at this temperature. The temperature is then allowed to rise during 30 minutes to 125° F., and further dyed at this temperature for 65 10 to 15 minutes. Then give 1 wash, 4 pas-

sages in sodium perborate, 2 lbs. per 100 gals. at 120° F., 2 cold washes, 5 passes in boiling soap solution 3 lbs. soap to 100 gallons, then rinse and wash in the open, dry and calender.

When using the dyestuff pastes according to our co-pending application, Serial No. 167,066, where the assistant is already in the color paste, the foregoing example is simplified to the extent indicated by the following process.

#### EXAMPLE II

An 8½% shade of Ponsol blue GD prepared according to said co-pending case on 150 lbs. mercerized cotton material.

12.75 lbs. of said vat color paste (containing 80 8.15 of assistant) are screened and poured into a bath composed of:

10 lbs. caustic soda (dry) 85

15 lbs. sodium hydrosulfite to

100 gallons bulk

and the dyeing process carried out as described above.

#### EXAMPLE III

##### Padding-jigger dyeing method

The padding liquor is composed of:

5 lbs. Ponsol blue GD prepared according to said co-pending case and containing 64% of the new assistant. 95

11½ gals. water

8 ozs. gum tragacanth

5 lbs. bleaching oil

100

12½ gallons bulk

The squeeze of the pad roller is about 60%. The padded material is then dried and developed in a jigger according to the process 105 of Example II above, by adding an additional quantity of the dyestuff paste so as to have an 8½% dyeing.

The developing bath contains the same ingredients in the same quantities as under 110 Example II, the dyeing being carried on under the same conditions. This process offers the advantage of better penetration and is usually adopted in the mills.

This process may be changed also as follows:

#### EXAMPLE IV

The pad liquor is composed of:

5 lbs. Ponsol blue GD (Schultz #842) or dark blue BR (Schultz #763) 120

11½ gals. water

8 ozs. gum tragacanth

5 lbs. bleaching oil

125

12½ gals. bulk

and the assistant added directly to the development bath, that is, for a shade corresponding to an 8½% shade of Ponsol blue GD a quantity of assistant equal to the amount of the dyestuff is used.

## EXAMPLE V

Package process:

5% shade of Ponsol dark blue BR (Schultz #763) or violet RRD (Schultz #766). The boiled off yarn is dyed in the package machine with:

5% of vat color paste  
 2½% caustic soda (dry)  
 3% sodium hydrosulfite  
 10 3% assistant  
 water

The conditions of dyeing are the same as usual. After dyeing rinse and oxidize with 2% sodium perborate, rinse, soap, rinse and dry.

If the vat color pastes prepared according to our co-pending case above are used, the above formula is modified as follows:

20 5% dyestuff prepared according to said co-pending application.  
 2½% caustic soda  
 3% sodium hydrosulfite  
 Water

25 The shades come out bright and very even. It is obvious that the preparing of the dye liquors from all the ingredients used may be varied by the dyer.

30 Advantages and results from the use of these assistants, either by direct addition to the dyebath or by preliminary addition to the vat dyestuff pastes:

35 1. The exhaust of these dyebaths are much better than those used at present, which accounts for an increased yield in depth of shade.

40 2. The effect of the assistant as an excellent solvent is shown in slowing down the rate at which the dye goes on, which results in equalizing the depth of dyeing giving, in this way, extremely even results. This is of very great advantage for dyes having great affinity such as blue GD, violet RRD, blue BCS, dark blue BR, etc.

45 3. The fixation of the dyestuff is improved over the results of the usual methods, therefore, on soaping in a boiling soap solution the dyestuff loses less which accounts for an increased yield in shade (depth).

50 4. Due to perfect dyeing conditions the brilliancy of the dyeing is enhanced.

55 5. It is well known that most of the dyes, when being treated with a soap solution change considerably in shade. This is the case, for example, with the indanthrene blues (Schultz #842) but when dyed according to this method, additional soaping does not change the shade to any noticeable extent.

60 6. The addition of the assistant to the dyestuff paste puts the latter in a perfectly dispersed condition permitting a much quicker screening (several hours economy in time) and permitting the padding of an absolutely speck free paste which is of enormous value

for the so-called pad-jigger dye process. It allows the dyer to obtain very uniform and speck free light shades which are not obtained today without great difficulty.

7. Pastes containing the new assistant do not dry out around the edge of the container. This is a very great advantage because the ordinary commercial pastes tend to dry out, the dry particles agglomerate and the result is specky dyeings when the color is used on piece goods. Actually to prevent this condition causes the dyer considerable trouble which is avoided by this invention.

8. The addition or presence in the vat paste of such assistant is particularly of great assistance when dyeing with vat dyestuffs of the very insoluble type such as the highly chlorinated indanthrene blues, etc. It always insures a perfect solution, regulates the exhaust and results in a very level dyeing.

As many apparently widely different embodiments of this invention may be made without departing from the spirit thereof, it is to be understood that we do not intend to limit ourselves to the specific embodiments thereof except as indicated in the appended claims.

We claim:

1. The process of improving a vat color paste, the step which comprises incorporating with the vat color paste a compound having the structural formula:



100

wherein  $\text{R}_1$ ,  $\text{R}_2$  represents either the alkyl group  $\text{C}_n\text{H}_{(2n+1)}$  hydrogen, or the hydroxy alkyl group  $\text{C}_n\text{H}_{2n}\text{OH}$ .

2. The process of improving a vat color paste, the step which comprises incorporating with the vat color paste a compound of the type described in claim 1, in which compound  $\text{C}_n\text{H}_{2n}\text{OH}$  represents the radical  $\text{C}_2\text{H}_4\text{OH}$ .

3. The process of improving a vat color paste, the step which comprises incorporating with the vat color paste a compound having the structural formula:



115

wherein  $\text{C}_n\text{H}_{2n}\text{OH}$  represents an aliphatic radical, substituted or not, and  $\text{R}_1$  and  $\text{R}_2$  represents either hydrogen or an aliphatic radical or a hydroxy-aliphatic radical.

4. The process of improving a vat color paste, the step which comprises incorporating with the vat color paste a compound of the type described in claim 3, wherein  $\text{R}_1$  represents a hydroxy-aliphatic radical.

5. The process of improving a vat color paste, the step which comprises incorporating with the vat color paste a compound of the type described in claim 3, wherein  $\text{R}_1$

125

130

represents a hydroxy-aliphatic radical and R<sub>2</sub> represents hydrogen.

6. The process of improving a vat color paste, the step which comprises incorporating with the vat color paste a compound of the type described in claim 3, wherein R<sub>2</sub> represents hydrogen.

7. The process of improving a vat color paste, the step which comprises incorporating with the vat color paste a compound of the type described in claim 3, in which compound both C<sub>n</sub>H<sub>2n</sub>OH and R<sub>1</sub> represent the radical C<sub>2</sub>H<sub>4</sub>OH.

8. In the process of dyeing with vat colors, the step which comprises incorporating in the vat a compound having the structural formula:



20 wherein R<sub>1</sub>, R<sub>2</sub> represents either the alkyl group C<sub>n</sub>H<sub>(2n+1)</sub> hydrogen, or the hydroxy alkyl group C<sub>n</sub>H<sub>2n</sub>OH.

9. In the process of dyeing with vat colors, the step which comprises incorporating in the vat a compound of the type described in claim 1, in which compound C<sub>n</sub>H<sub>2n</sub>OH represents the radical C<sub>2</sub>H<sub>4</sub>OH.

10. In the process of dyeing with vat colors, the step which comprises incorporating in the vat a compound having the structural formula:



35 wherein C<sub>n</sub>H<sub>2n</sub>OH represents an aliphatic radical, substituted or not, and R<sub>1</sub> and R<sub>2</sub> represents either hydrogen or an aliphatic radical or a hydroxy-aliphatic radical.

40 11. In the process of dyeing with vat colors, the step which comprises incorporating in the vat a compound of the type described in claim 3, wherein R<sub>1</sub> represents a hydroxy-aliphatic radical.

45 12. In the process of dyeing with vat colors, the step which comprises incorporating in the vat a compound of the type described in claim 3, wherein R<sub>1</sub> represents a hydroxy-aliphatic radical and R<sub>2</sub> represents hydrogen.

50 13. In the process of dyeing with vat colors, the step which comprises incorporating in the vat a compound of the type described in claim 3, wherein R<sub>2</sub> represents hydrogen.

55 14. In the process of dyeing with vat colors, the step which comprises incorporating in the vat a compound of the type described in claim 3, in which compound both C<sub>n</sub>H<sub>2n</sub>OH and R<sub>1</sub> represent the radical C<sub>2</sub>H<sub>4</sub>OH.

In testimony whereof we affix our signatures.

JEAN GEORGES KERN.  
CHARLES J. SALA.

**Certificate of Correction**

Patent No. 1,782,122.

Granted November 18, 1930, to

JEAN GEORGES KERN ET AL.

It is hereby certified that error appears in the printed specification of the above numbered patent requiring correction as follows: Page 1, line 90, strike out the formula and insert instead  $C_nH_{(2n-1)}(OH)_2$ ; page 3, lines 115 to 117, strike out the formula and insert instead  $\begin{array}{c} /C_nH_{2n}OH \\ N-R_1 \\ \backslash R_2 \end{array}$ ; and that the said Letters Patent should be read with these corrections therein that the same may conform to the record of the case in the Patent Office.

Signed and sealed this 23d day of December, A. D. 1930.

[SEAL.]

M. J. MOORE,  
*Acting Commissioner of Patents.*